

# UNITED STATES PATENT OFFICE.

EDWARD H. ELLIS, OF SOMERVILLE, MASSACHUSETTS, ASSIGNOR, BY MESNE ASSIGNMENTS, TO SAID EDWARD H. ELLIS, AND ALFRED D. CHANDLER, OF BROOKLINE, MASSACHUSETTS, TRUSTEES OF ELLIS BRIQUET BINDER.

## FUEL-BRIQUET AND METHOD OF MAKING SAME.

1,009,960.

Specification of Letters Patent. Patented Nov. 28, 1911.

No Drawing.

Application filed January 18, 1911. Serial No. 603,382.

To all whom it may concern:

Be it known that I, EDWARD H. ELLIS, of Somerville, in the county of Middlesex and State of Massachusetts, have invented certain new and useful Improvements in Fuel-Briquets and Methods of Making Same, (Case A,) of which the following is a specification.

This invention relates to a new and useful briquet as an article of manufacture, and to the particular application of the process for making such new and useful briquet.

Heretofore the best briquets have been made with binders of coal tar pitch, or of silicates, and of oil, but the smoke and the odor from such binders have impaired their usefulness and sale.

This invention provides a fuel briquet free from the aforesaid objections, and which is cohesive, waterproof, odorless, smokeless, retains its form in the fire, has a high calorific efficiency, and is comparatively inexpensive to manufacture.

In carrying out my invention, I first produce a composition containing sulfuric acid, molasses and water, or their reaction products. This composition is then incorporated with comminuted fuel and the composition is then mechanically pressed into the form of briquets; the briquets are then subjected to calorific action of a certain temperature through the medium of a specially designed and regulated oven.

The composition may be in the proportions of three (3) lbs. of sulfuric acid, preferably of a concentration in excess of ninety per cent., one (1) gallon of molasses and three (3) gallons of water, this total quantity of composition being then used in the proportions of one hundred and twenty-five (125) lbs. of composition to one (1) ton of comminuted fuel. I do not, however, limit myself to these specific proportions, and any chemical equivalent of molasses may be employed, instead of commercial molasses. When the composition and fuel have been thoroughly incorporated by suitable machinery, the briquets are made into any desired form, preferably under such a pressure as the graded requirements of combustion demand. The briquets are then subjected to a process of final elimination of moisture, and simultaneously to a process of

induration and waterproofing, through the added binding operation of calorific upon the chemical ingredients employed in the composition, these effects being produced by a suitably arranged oven kept at a temperature of about two hundred (200°) F. and through which the passage of the briquets is regulated for from ten (10) to about fifteen (15) minutes, the degree of the heat and the duration of the transit in the oven being governed by the kind of service for which the briquets are intended. Under these conditions the carbohydrates of the molasses undergo dehydration and carbonization at comparatively low temperatures in presence of the sulfuric acid, with the result that an insoluble, strong, rigid and highly efficient binder is formed throughout the mass of the fuel. I have found in practice that such briquets are not only hard enough to bear transportation and handling, but that they are also waterproof, and are odorless and smokeless during combustion. Also, that they possess a high calorific efficiency and preserve their form in the fire, the outer portion during combustion presenting of course some ash, which, however, is crowded off, but leaving the inner and unconsumed portions still hard enough to sustain the weight of fresh fuel above, and to preserve their form during "slicing" of the fire.

One of the chief reasons why my improved briquets are economical to manufacture is that the chemicals specified so combine as to reduce to the minimum the time and degree of heat applied to render them hard and waterproof, the carbonization of the carbohydrates of the molasses by the sulfuric acid occurring at a comparatively low temperature.

Comminuted bituminous or soft coal made into briquets with my improved composition and treatment, is as hard as anthracite coal, and burns without the annoying smoke nuisance usually resulting from the use of soft coal.

Briquets manufactured under my invention have the equivalent weight value of hard coal, but without cinder loss because of the complete combustion of the briquets.

I claim:

1. A waterproof briquet manufactured of

105

commminuted fuel and a composition includ-  
ing an insoluble, carbonized reaction prod-  
uct of sulfuric acid, and molasses.

2. A waterproof briquet manufactured of  
5 commminuted fuel mixed with a composition  
containing an insoluble, carbonized reaction  
product of sulfuric acid, molasses and wa-  
ter, the said fuel and composition being  
mixed, shaped and baked.
- 10 3. A waterproof briquet manufactured of  
commminuted fuel, and an insoluble, carbon-  
ized reaction product of sulfuric acid and  
molasses rendered hard and waterproof by  
heat.
- 15 4. The method of making waterproof fuel

briquets, consisting in mixing with com-  
minuted fuel a composition containing an  
insoluble, carbonized reaction product of  
sulfuric acid, molasses and water, forming  
the mixture into briquets under pressure, 20  
and then subjecting the briquets to the ac-  
tion of heat to render them hard and water-  
proof.

In testimony whereof I have affixed my  
signature, in presence of two witnesses.

EDWARD H. ELLIS.

Witnesses:

A. W. HARRISON,  
E. BATCHELDER.